# EUROPEAN PATENT SPECIFICATION

(11) **EP 0 526 556 B1**
(45) Date of publication and mention of the grant of the patent: **26.08.1998**
(21) Application number: 91908818.7
(22) Date of filing: 26.04.1991
(51) Int. Cl.: H01B 3/44, C08L 27/18, C08L 29/10

(54) **ELECTRICAL INSULATING MATERIAL**
ELEKTRISCHES ISOLATIONSMATERIAL
MATERIAU D'ISOLATION ELECTRIQUE

(30) Priority: 27.04.1990 GB 9009407; 27.04.1990 US 515302
(43) Date of publication of application: 10.02.1993
(62) Divisional of application: 92202891.5
(73) Proprietor: W.L. GORE & ASSOCIATES, INC., Newark, Delaware 19714-9206 (US); W.L. GORE & ASSOCIATES (UK) LTD, London WC2A 2JP (GB)
(72) Inventor: GELLAN, Andrea, Dunfermline KY12 7QP (GB); MORTIMER, William, Patrick, Jr., Conowingo, MD 21918 (US)
(74) Representative: Horner, Martin Grenville
(86) International application number: GB9100661
(87) International publication number: WO9117551

(56) References cited:
- EP-A- 0 010 152
- EP-A- 0 138 524
- US-A- 3 484 503
- US-A- 4 128 693
- US-A- 4 454 249

## Description

### TECHNICAL FIELD

The present invention relates to an electrical insulating composite material which is extruded and calendered to form a tape and particularly though not exclusively, used for insulating wire. The invention also includes a process for preparing the composite tape material, and to an insulated conductor.

### DESCRIPTION OF PRIOR ART

The use of polytetrafluoroethylene (PTFE) or copolymers formed from tetrafluoroethylene (TFE) and perfluoro (propyl vinyl ether) (PPVE) is well known for the insulation of wire. These polymers have good heat resistance, high resistance to solvent attack and good dielectric properties. These attributes are desirable where high reliability is required, for example in aerospace applications.

Other desirable attributes for such applications include mechanical properties such as resistance to abrasion and resistance to cut-through of insulation by sharp edges. However, the properties of the aforesaid materials are poor in these respects.

Attempts have been made in the past to improve the mechanical properties of TFE base polymers by including additives such as glass spheres, silica flake, etc. However, the improvements achieved with such compositions are generally limited and often at the expense of other desirable features, for example leading to degradation of electrical properties or mechanical properties such as flexibility.

Attempts have also been made in the past to improve the mechanical properties of the fluoropolymers by mixing with other polymers having better mechanical properties, such as polyphenylene sulphide, polyphenylene oxide, etc. However, these other polymers are in general incompatible with fluoropolymers so that there is difficulty in producing intimate blends.

US 4 128 693 relates to a wire coated with a fluorocarbon composite material. The material is extruded directly onto the wire and not calendered into a tape.

US 4 454 249 relates to a reinforced plastic which is moulded from a resin matrix such as stretched PTFE. The material is intended to be used as a moulding composition and is not extruded or calendered into a tape.

EP 0 138 524 describes a specialised composition which includes irradiated PTFE. The composition is melt extruded to provide an insulating layer on a conductor.

EP 0 010 152 discloses the use of mixes of PTFE and copolymer. The mixture is not extruded or calendered into a tape.

US 348 503 relates to blends of fluorinated polymers. The document is directed to blends containing 50 to 90 weight percent of a copolymer of tetrafluoroethylene and perfluoro(alkyly vinyl ether).

GB 2 262 101 relates to a composite sheet material composed of a porous membrane of expanded polytetrafluoroethylene (PTFE) and a thermoplastic copolymer of tetrafluoroethylene and perfluoro(propylvinylether). The composite that comprises 5 to 95 wt% of copolymer, at least a portion of which is entrapped within the pores of the porous membrane.

It is among the objects of embodiments of the present invention to mitigate at least one of the problems mentioned above.

### SUMMARY OF THE INVENTION

In accordance with a first aspect of the present invention, there is provided an electrically insulating composite material comprising in the form of a tape and comprising an intimate admixture of 5 to 40 wt.% of a thermoplastic copolymer of tetrafluoroethylene and perfluoro(propylvinylether) and 60 to 95 wt.% of coagulated dispersion type polytetrafluoroethylene (PTFE) ; the composite material having been extruded and calendered to form the tape.

The tape of the present invention is non-porous.

Preferably the electrically insulating composite material comprises 8 to 20 wt% of copolymer and 80 to 92 wt% of PTFE.

Most preferably, the non-porous material typically has a density of 2.0 to 2.2 g/cm³.

In order to produce the composite material, the thermoplastic copolymer of tetrafluoroethylene and perfluoro(propylvinylether) [TFE/PPVE copolymer] is preferably used in particulate form and preferably has a particle size in the range 1 to 180 microns, especially 20 to 100 microns. The particles may have a wide range of particle sizes and preferably include particles having sizes right across the ranges. However, particles of narrow size range may also be used. The TFE/PPVE copolymer particles preferably have a substantially regular shape, such as oblong or spherical.

The polytetrafluoroethylene component is of the coagulated dispersion type. As is well known, polytetrafluoroethylene (PTFE) can be produced in three quite distinct forms having different properties viz; granular PTFE, coagulated dispersion PTFE, and liquid PTFE dispersions. Coagulated dispersion PTFE is also referred to as fine powder PTFE. In the present invention, the PTFE resin can be used in powder form; or alternatively, the PTFE resin can be coagulated from an aqueous dispersion in the presence of perfluoroalkoxy TFE/PVE copolymer powder or dispersion. The coagulation of PTFE in the presence of a dispersion of the copolymer results in a co-coagulation of PTFE and copolymer. The flocculated mixture may then be decanted and dried.

The composite material may be used for producing a covering for wire, or other electrically conductive substrate; for example, one to which bonding is not normally required.

In accordance with a second aspect of the present invention there is provided an insulated electrical conductor which comprises a wire having an electrically insulating layer formed of the composite material of the present invention around the wire.

Usually the composite material is wrapped around the wire in overlapping turns. The overlapping areas of the material may then be fused together, for example at temperatures of 350 to 450°C (for 0.5 to 20 minutes). The time will be in correspondence with the temperature employed. Lower temperatures tend to minimise degradation of the material. The time and temperature conditions also depend on the construction of the insulated conductor, such as thickness of the insulation and number of cores in the wire.

It has been found that wire electrical insulation made from wrapped and sintered tape produced from the composition has an unexpectedly better cut-through resistance and abrasion resistance than equivalent wire insulation made from fine powder PTFE alone.

In accordance with a third aspect of the present invention there is provided an insulated electrical conductor which comprises a wire having wrapped around it at least two adjacent layers, one layer being formed of the non-porous composite material of the present invention, and the second layer being formed of porous composite sheet material; the porous material being formed of a porous membrane of expanded polytetrafluoroethylene (PTFE) and a thermoplastic copolymer of tetrafluoroethylene and perfluoro(propylvinylether), wherein at least a portion of the thermoplastic copolymer is entrapped within the pores of the porous polytetrafluoroethylene.

Generally, the layers are applied in the form of tapes wrapped (preferably counter-wrapped) around the wire in overlapping turns. The layers may also be applied longitudinally with a longitudinal overlapping seam. Preferably, sintering takes place after the two tapes have been applied; so that the layers become fused into an integral structure. Sintering may be brought about under the conditions previously described.

The second layer of porous composite sheet material may be prepared by mixing a thermoplastic copolymer of tetrafluoroethylene and perfluoro(propylvinylether) with a dispersion of the coagulated fine powder polytetrafluoroethylene resin or with a dispersion of the fine powder and coagulating the solids to obtain a resin blend, preparing pellets of the resin blend, forming a tape from the pellets and stretching the tape until a desired degree of porosity is attained. Preferably, the composite sheet material is prepared from a flocculated mixture of the TFE/PPVE copolymer and PTFE, in particulate form. The mixture is lubricated for paste extrusion with an ordinary lubricant known for use in paste extrusion, and pelletized. The pellets are preferably aged at 40-60°C and are then paste extruded into a desired shape, usually a film. The extruded shape is then stretched, preferably in a series of at least two stretch steps while heating at between 35-360°C until a desired degree of porosity is attained. The porosity occurs through the formation of a network of interconnected nodes and fibrils in the structure of the stretched PTFE film, as more fully described in U.S. Patent 3,953,566. The density of the porous material will usually be less than 2.0 g/cc.

At the stretch temperatures employed, the TFE/PPVE copolymer melts and, depending on the amount present, may become entrapped in the pores or nodes formed, may coat the nodes or fibrils, or may be present on the outer surface of the membrane formed. Most likely a combination of each embodiment occurs, depending on whether the copolymer and the PTFE remain as distinct moieties.

The porous composite sheet material is useful as an insulation covering for wire and cable, particularly in electrical applications. It is believed that the presence of the TFE/PPVE copolymer aids in adhering the layers of tape wrap to one another. The composite sheet material can be sintered either before or after wrapping if desired to improve cohesiveness and strength of the material per se. Once the composite sheet material has been prepared, it can be compressed, if desired, to increase the density of the composite. Such compression does not significantly affect the increased matrix strength that is associated with expanded porous PTFE. Compression improves properties such as dielectric strength and cut-through resistance.

The porous composite sheet material has good cut-through resistance, strength and abrasion resistance.

Examples of porous composite sheet materials suitable for use in conjunction with the present invention are disclosed in the present application, and in our British patent application GB2,262,101.

It has been found that generally speaking the non-porous composite tape material of the present invention has good electrical (particularly dielectric) properties; whilst the porous composite sheet material (whether compressed after expansion or not) has good mechanical properties (particularly cut-through resistance).
Surprisingly these properties are retained in the two-layer insulated electrical conductor notwithstanding sintering, so that an insulating layer having both good mechanical and electrical properties is obtained. Either the porous or the non-porous layer may be adjacent the wire. Placing the non-porous layer of the present invention adjacent the wire facilitates stripping of the wire when a connection is to be made. Placing the non-porous layer uppermost allows better overprinting (e.g. for colour coding).

If required more than two layers of material may be used, for example non-porous/porous/non-porous which provides good stripping and printing characteristics.

Also, one or more porous or non-porous layers of the material of the present invention may be wrapped together with one or more layers of conventional expanded or non-expanded PTFE tape prior to sintering. In particular, the combination of layers of non-porous composite tape material with conventional expanded PTFE may be used.

In accordance with a fourth aspect of the present invention there is provided a method of insulating an electrical conductor comprising;
paste extruding an electrically insulating material formed from an intimate mixture of 5 to 40 weight percent of a particulate thermoplastic copolymer of tetrafluoroethylene and perfluoro (propyl vinyl ether); and
60 to 95 weight percent of coagulated dispersion type polytetrafluoroethylene; calendering the material and forming a tape; applying said tape around an electrically conductive substrate; and sintering the material before or after application to the substrate.

The paste extrusion step may be carried out using conventional PTFE extrusion techniques (for example in admixture with a liquid carrier, such as a hydrocarbon). The extruded composition is generally of thin section so as to allow efficient removal of the liquid carrier and formation of a solid material, usually in the form of a sheet, tape or filament. The solid material is mechanically worked, by calendering, to modify its shape or thickness prior to application to the substrate.

In accordance with a fifth aspect of the present invention, there is provided a method of insulating an electrical conductor which comprises wrapping two adjacent layers of tape of composite material around a wire, one layer being formed of non-porous composite material of the present invention and the second layer being formed of porous composite sheet material; the porous material being formed of a porous membrane of expanded polytetrafluoroethylene (PTFE) and a thermoplastic copolymer of tetrafluoroethylene and per fluoro(propylvinylether), wherein at least a portion of the thermoplastic copolymer is entrapped within the pores of the porous polytetrafluoroethylene and sintering the material to fuse the layers into a unitary structure.

### EXAMPLES

Embodiments of the present invention will now be described in Examples 1, 2, 6, 7, 8 and 9 by way of example only. Examples 3 to 5 relate to composite sheet materials which are claimed in our UK patent GB 2,262,101. The Examples have been included in the present specification for illustrative purposes as the processes described therein may be applied to embodiments of the present invention.

Figure 1 shows a wire construction.

### EXAMPLE 1 (non-porous tape)

81g (9wt %) of the TFE/PPVE copolymer powder of wide particle size distribution which had been screened to a particle size in the range 1-150 microns was added to 1.81kg (91wt %) of Hostaflon (Registered Trade Mark) 2023 PTFE resin powder and tumbled in a Pascall tumble mixer at 40 revs/min for 60 minutes. 620 ml of Shellsol (Registered Trade Mark) TD liquid hydrocarbon was then added to this powder mixture and tumbled for a further 30 minutes to form a paste.
The paste was then left overnight before being compressed at 200 psi (14.06 kg/cm²) into a 4 inch (10.2cm) diameter pellet. The pellet was left for 24 hours at a temperature of 35 to 39°C before extrusion on a standard PTFE ram extruder at room temperature.

The extrudate of thickness 0.035 inch (890 microns) was then calendered down to 0.004 inch (101 microns) in three stages, using rollers heated to approximately 50°C. The 0.004 inch (100 microns) tape was slit and wrapped on to 22 AWG (American Wire Gauge) 19 strand silver plated electrical wire conductor, to an insulation wall thickness of 0.008 inch (200 microns) and sintered in air at 400°C for 0.5 minute.

A similar wire sample was made using only the PTFE resin for comparison.

Both wire samples were tested for dynamic cut-through resistance and scrape abrasion resistance according to the test method given in BS G 230 (British Standard, Group 230). The results are given in Table 1 and demonstrate the improvement in the mechanical performance of the PTFE wire insulation when blended with TFE/PPVE copolymer over and above that of the base PTFE resin.

**Table 1**

| DYNAMIC CUT THROUGH SCRAPE ABRASION (4 Newtons Load) in Newtons (N) | | |
|---|---|---|
| SAMPLE | (Room Temperature) | (Room Temperature) |
| A | 63 | 2,000 cycles |
| B (comparison) | 28 | 200 cycles |
| Sample A: 22 AWG, 19 strand, silver plated copper conductor with 0.008 inch (200 microns) wall of PTFE and TFE/PPVE blended insulation material. (according to Example 1). | | |
| Sample B: 22 AWG, 19 strand, silver plated copper conductor with 0.008 inch (200 microns) wall of PTFE insulation. | | |

### EXAMPLE 2 (non-porous tape)

1.2Kg of TFE/PPVE copolymer powder of particle size was dispersed in 3.75Kg of Shellsol (Trademark) TD liquid hydrocarbon.

This was achieved by grinding the suspension in a colloid mill down to approximately 0.002 inch (50 microns ± 12 microns). The resultant slurry was added to 13.61Kg of Hostaflon (Trade mark) 2023 PTFE resin and tumbled for 7 minutes.

The powder/lubricant mixture was then compressed into a 4 inch pellet. Tape of thickness 0.003 inch (75 microns) was made from the resultant pellet by a similar method to that described in Example 1.

### EXAMPLE 3 (expanded tape)

302g. (16.7 wt.%) of a tetrafluoroethylene/perfluoro(propyl vinyl ether) copolymer powder (PFA powder) was added to 1.5 liters of methanol and diluted with 20.1 liters of deionized water to form a dispersion. This was mixed for 30 seconds in a baffled 5 gallon container.

Next, 6500g. of aqueous dispersion containing 1600g. (12.8 wt.%) of dispersion-produced polytetrafluoroethylene was mixed with the PFA powder dispersion. Then, 6.4g. polyethylene imine was added to coagulate the solids from the mixture. After about 20 seconds of stirring, the phases separated. The clear liquid was decanted and the remaining solids dried at 160°C for 24 hours. The solids, in particulate form, were lubricated with mineral spirits (19% by weight) and pelletized under vacuum. The pellets were aged at 49°C for about 24 hours, and were then extruded into tape. The tape was calendared to a thickness of 16.5 mil. and then dried to remove lubricant.

The dried tape was stretched in three steps. In the first stretch step, the tape was expanded longitudinally 93% (1.93 to 1) at 270°C at an output rate of 105 feet per minute (32m/min). In the second step, the tape was expanded longitudinally at a rate of 20:1 at 290°C at an output rate of 3.8 feet per minute (1.16m/min). In the third step, the tape was expanded longitudinally at a ratio of 2:1 at 325°C at an output of 75 feet per minute (23m/min).

The resulting porous tape was then subjected to heat at 330°C for about 6 seconds.

It was then compressed to almost full density. The bulk density was 2.0 gm/cc.

### EXAMPLE 4 (expanded tape)

The procedure of Example 3 was followed, except that in the first stretch step the stretch was at 1.9 to 1 instead of 1.93 to 1, and in the second stretch step the temperature was 300°C, and, in the third stretch step, the temperature was 360°C.

The tape was not compressed. The resulting density was 0.7 gm/cc.

### EXAMPLE 5 (mechanical properties)

Expanded tapes produced by the method given in Example 3 that had been compressed to almost full density to a thickness of 0.0007 inch (18 microns) were slit and wrapped onto 20 AWG, 19 strand silver plated electrical wire conductor, to an insulation wall finished thickness of 0.003 inch (75 microns) post-sinter.

The insulated wire was then heat treated in air at 350°C for 15 minutes, to fuse the insulation material.

The resultant wire was tested for dynanmic cut-through resistance according to the test method given in BS G 230.

BS G 230 (British Standard Group 230) is a test specification for general requirements for aircraft electrical cables. Test results are given in Table 2.

**Table 2.**

| Sample | Dynamic Cut-Through in Newtons (N) at Room Temperature |
|---|---|
| 20 AWG, 19 strand, | 91 |
| silver plated copper | 92 |
| conductor, with 0.003 inch (75 microns) | 65 |
| wall of fused insulation | 89 |
| tape. | Average = $\overline{\text{84}}$ |

### EXAMPLE 6 (mechanical properties)

The expanded tape made by the method given in Example 3 was slit and a 0.15mm thick layer (0.lmm post-sinter) was wrapped (layer A) on to 20 AWG (American Wire Gauge) 19 strand nickel plated copper conductor (C).

Tape made by the method given in Example 2 was slit and then a 0.20mm thick layer (0.15mm post-sinter) was counter-wrapped (layer B) on the above insulated wire (See Figure 1). Counter-wrapping means that the tapes were wound as spirals of opposite hand.

The resultant composite wire was then sintered in air at 400°C for 1.5 minutes. The insulation had a final post-sinter thickness of 0.25mm. Similar insulated wires were made with only the tape manufactured as in Example 3 or Example 4.

For the purposes of comparison, separate samples of conductor were insulated with standard PTFE or with TFE/PPVE jackets (Samples 1 and 2 respectively).

The overall diameter of all samples was maintained at 1.5mm, resulting in similar wall thicknesses to allow the samples to be compared with one another.

The mechanical properties, with respect to scrape abrasion and cut through resistance of the insulated wire samples, were measured according to the test method given in BS G 230. The results are given in Table 3 and show the overall improvement in the mechanical properties of the composite insulation materials when compared with the individual homogeneous insulation materials.

**Table 3**

| | DYNAMIC CUT THROUGH in Newtons (N) | SCRAPE ABRASION | |
|---|---|---|---|
| | | 8 Newtons Load | 4 Newtons Load |
| Sample | Room Temperature | (Room Temperature) | |
| 1 (comparison) | 35 | 12 | 310 |
| 2 (comparison) | 45 | 46 | 610 |
| 3 | 56 | 54 | 1,900 |
| 4 | 115 | 66 | 260 |
| 5 | 81 | 120 | 10,000 |

### Sample 1

20AWG, 19 strand, nickel plated copper conductor with 0.25mm wall of PTFE insulation.

### Sample 2

20AWG, 19 strand, nickel plated copper conductor with 0.25mm wall of TFE/PPVE insulation.

### Sample 3

20AWG, 19 strand, nickel plated copper conductor with 0.25mm wall of PTFE and TFE/PPVE blended insulation material (according to Example 2).

### Sample 4

20AWG, 19 strand, nickel plated copper conductor with 0.25mm wall of (expanded and densified) PTFE and TFE/PPVE blended insulation material (according to Example 3).

### Sample 5

20AWG, 19 strand, nickel plated copper conductor with 0.25mm wall of composite insulation consisting of 0.lmm of PTFE and TFE/PPVE blended material (according to Example 3) and 0.15mm PTFE and TFE/PPVE blended material (according to Example 2) fused together.

### EXAMPLE 7 (electrical performance)

When Samples 4 and 5, manufactured by the method given in Example 5 are subject to the High Voltage Immersion Test given in BS G 230, Test Method 16a, the following test results are obtained:

| | |
|---|---|
| Sample 4 | 3.5 KV |
| Sample 5 | 5 KV |

From these test results it is apparent that Sample 5, containing the dual counter-wrapped tapes manufactured by the methods given in Examples 2 and 3, has improved electrical properties with respect to voltage withstand characteristics over and above that of Sample 4.
Thus, for overall mechanical and electrical performance the dual, counter-wrapped construction is the preferred construction.

### EXAMPLE 8 (expanded/non-porous dual wrap)

Expanded tape made by the method given in Example 3 was slit and a 50 microns thick (post-sinter thickness) layer (A) was wrapped onto 20AWG (American Wire Gauge) 19 strand nickel plated copper conductor (C)..
Tape made by the method given in Example 2 was slit and a 150 microns thick (post-sinter thickness) layer (B) was then counter-wrapped on the above insulated wire.
The resultant composite wire was then fused by heat treatment in air at 350°C for 20 minutes.
Figures of 113 - 151 cycles to failure (8 Newton load), and 110 - 130 Newtons were obtained when tested respectively, at room temperature, for scrape abrasion and dynamic cut-through resistance, according to Test Methods 30 and 26 given in BS G 230.

### EXAMPLE 9 (non-porous/expanded dual wrap)

Tape made by the method given in Example 2 was slit and a 150 microns thick (post-sinter thickness) layer (A) was wrapped onto 20AWG (American Wire Gauge) 19 strand nickel plated copper conductor (C).
Expanded tape made by the method given in Example 3 was slit and a 50 microns thick (post-sinter thickness) layer (8) was counter-wrapped on the above insulated wire.
The resultant composite wire was then fused by heat-treatment in air for 1.5 minutes at 400°C followed by 20 minutes at 350°C.
When tested to Test Methods 16a, 26 and 30 in BS G 230, the results in Table 4 were obtained.

**Table 4**

| Test | Test Method | Result |
|---|---|---|
| High Voltage | BS G 230 | 5 KV |
| Immersion Test | Test 16a | |
| Dynamic Cut-Through | BS G 230 | 139 N |
| | Test 26 | |

| | (Room Temperature) | |
|---|---|---|
| Scrape Abrasion | BS G 230 | 95 Cycles |
| | Test 30 | |
| | (8N Load, Room Temperature) | |

## Claims

1. An electrically insulating composite material in the form of a tape and comprising an intimate admixture of 5 to 40 wt.% of a thermoplastic copolymer of tetrafluoroethylene and perfluoro(propylvinylether) and 60 to 95 wt.% of coagulated dispersion type polytetrafluoroethylene (PTFE); the composite material having been extruded and calendered to form the tape.

2. A material according to claim 1 which comprises 8 to 20 wt.% of copolymer, and 80 to 92 wt.% of PTFE.

3. A material according to claim 1 or 2 which has a density of 2.0 to 2.2 g/cc.

4. An insulated electrical conductor which comprises a wire (C) having an electrically insulating layer (A) formed of a tape according to claim 1 around the wire.

5. A conductor according to claim 4 wherein the tape has been sintered.

6. An insulated electrical conductor which comprises a wire (C) having wrapped around it at least two adjacent layers (A, B), one layer being formed of non-porous composite material according to claim 1, and the second layer being formed of porous composite sheet material; the porous material being formed of a porous membrane of expanded polytetrafluoroethylene (PTFE) and a thermoplastic copolymer of tetrafluoroethylene and perfluoro (propylvinylether), wherein at least a portion of the thermoplastic copolymer is entrapped within the pores of the porous polytetrafluoroethylene.

7. An insulated conductor according to claim 6 wherein the non-porous layer is adjacent the wire, and the porous layer overlies the non-porous layer.

8. An insulated conductor according to claim 6 wherein the porous layer is adjacent the wire, and the non-porous layer overlies the porous layer.

9. An insulated conductor according to claim 6, 7 or 8 which has been sintered to fuse the layers of composite material.

10. A method of insulating an electrical conductor comprising paste extruding an electrically insulating material formed from an intimate mixture of 5 to 40 wt.% of a particulate thermoplastic copolymer of tetrafluoroethylene and perfluoro(propylvinylether), and 60 to 95 wt.% of coagulated dispersion type polytetrafluoroethylene; calendering the material and forming a tape; applying said tape around an electrically conductive substrate; and sintering the material before or after application to the substrate.

11. A method according to claim 10 wherein the material is sintered at 350 to 450°C for a time of 0.5 to 20 mins.

12. A method of insulating an electrical conductor which comprises wrapping two adjacent layers of tape of composite material around a wire, one layer being formed of non-porous composite material according to claim 1 and the second layer being formed of porous composite sheet material; the porous material being formed of a porous membrane of expanded polytetrafluoroethylene (PTFE) and a thermoplastic copolymer of tetrafluoroethylene and perfluoro (propylvinylether), wherein at least a portion of the thermoplastic copolymer is entrapped within the pores of the porous polytetrafluoroethylene and sintering the material to fuse the layers into a unitary structure.

## Patentansprüche

1. Elektrisch isolierendes Verbundmaterial in Form eines Bandes, umfassend ein inniges Zugemisch von 5 bis 40 Gew.-% eines thermoplastischen Copolymers von Tetrafluorethylen und Perfluor(Propylvinylether) und 60 bis 95 Gew.-% Polytetrafluorethylen (PTFE) als koagulierte Dispersion, wobei das Verbundmaterial zur Bildung des Bandes extrudiert und kalandriert wurde.

2. Material nach Anspruch 1, umfassend 8 bis 20 Gew.-% Copolymer und 80 bis 92 Gew.-% PTFE.

3. Material nach Anspruch 1 oder 2, welches eine Dichte von 2,0 bis 2,2 g/cm³ aufweist.

4. Isolierter elektrischer Leiter, mit einem Draht (C), der eine elektrisch isolierende Schicht (A) in Form eines Bandes gemäß Anspruch 1 aufweist, die den Draht umgibt.

5. Leiter nach Anspruch 4, bei dem das Band gesintert wurde.

6. Isolierter elektrischer Leiter, umfassend einen Draht (C), um den herum mindestens zwei benachbarte Schichten (A, B) gewickelt sind, von denen eine Schicht aus einem nicht-porösen Verbundmaterial gemäß Anspruch 1 gebildet ist, und die zweite Schicht aus einem porösen Verbund-Flachmaterial gebildet ist, wobei das poröse Material hergestellt ist aus einer porösen Membran aus expandiertem Polytetrafluorethylen (PTFE) und einem thermoplastischen Copolymer von Tetrafluorethylen und Perfluor(Propylvinylether), wobei mindestens ein Teil des thermoplastischen Copolymers in den Poren des porösen Polytetrafluorethylens gefangen ist.

7. Isolierter Leiter nach Anspruch 6, bei dem die nicht-poröse Schicht dem Draht benachbart ist und die poröse Schicht über der nicht-porösen Schicht liegt.

8. Isolierter Leiter nach Anspruch 6, bei dem die poröse Schicht dem Draht benachbart ist und die nicht-poröse Schicht über der porösen Schicht liegt.

9. Isolierter Leiter nach Anspruch 6, 7 oder 8, der gesintert wurde, um die Schichten des Verbundmaterials zu verschmelzen.

10. Verfahren zum Isolieren eines elektrischen Leiters, umfassend das Pastenextrudieren eines elektrisch isolierenden Materials, welches gebildet wurde aus einem innigen Gemisch von 5 bis 40 Gew.-% eines teilchenförmigen thermoplastischen Copolymers von Tetrafluorethylen und Perfluor(Propylvinylether) und 60 bis 95 Gew.-% Polytetrafluorethylen in Form einer koagulierten Dispersion; Kalandrieren des Materials und Bilden eines Bandes; Aufbringen des Bandes auf ein elektrisch leitendes Substrat; und Sintern des Materials vor oder nach dem Aufbringen auf das Substrat.

11. Verfahren nach Anspruch 10, bei dem das Material bei 350 bis 450°C während 0,5 bis 20 Minuten gesintert wird.

12. Verfahren zum Isolieren eines elektrischen Leiters, umfassend das Umwicklen eines Drahts mit zwei benachbarten Bandschichten aus Verbundmaterial, wobei eine Schicht aus einem nicht-porösen Verbundmaterial gemäß Anspruch 1 und die zweite Schicht aus einem porösen Verbund-Flachmaterial gebildet ist; wobei das poröse Material gebildet ist aus einer porösen Membran aus expandiertem Polytetrafluorethylen (PTFE) und einem thermoplastischen Copolymer von Tetrafluorethylen und Perfluor(Propylvinylether), wobei mindestens ein Teil des thermoplastischen Copolymers in den Poren des porösen Polytetrafluorethylens gefangen ist, und das Material gesintert wird, um die Schichten zu einer einheitlichen Struktur zu verschmelzen.

## Revendications

1. Matériau composite d'isolation électrique sous forme d'un ruban, comprenant un mélange intime de 5 à 40% en poids d'un copolymère thermoplastique de tétrafluoroéthylène et de perfluoro(propylvinyléther) et de 60 à 95% en poids de polytétrafluoroéthylène (PFTE) de type dispersion coagulée; le matériau composite ayant été extrudé et calandré pour former le ruban.

2. Matériau selon la revendication 1, qui comprend 8 à 20% en poids de copolymère et 80 à 92% en poids de PFTE.

3. Matériau selon la revendication 1 ou 2, qui a une masse volumique de 2,0 à 2,2 g/cm³.

4. Conducteur électrique isolé qui comprend un fil (C) portant une couche d'isolation électrique (A) formée d'un ruban selon la revendication 1 autour du fil.

5. Conducteur selon la revendication 4, dans lequel le ruban a été fritté.

6. Conducteur électrique isolé, qui comprend un fil (C) revêtu d'au moins deux couches adjacentes (A, B), une couche étant formée d'un matériau composite non poreux selon la revendication 1, et la seconde couche étant formée d'un matériau composite poreux en feuille; le matériau poreux étant formé d'une membrane poreuse de polytétrafluoroéthylène (PFTE) expansé et d'un copolymère thermoplastique de tétrafluoroéthylène et de perfluoro(propylvinyléther), dans lequel au moins une partie du copolymère thermoplastique est noyée à l'intérieur des pores du polytétrafluoroéthylène poreux.

7. Conducteur isolé selon la revendication 6, dans lequel la couche non poreuse est adjacente au fil, et la couche poreuse recouvre la couche non poreuse.

8. Conducteur isolé selon la revendication 6, dans lequel la couche poreuse est adjacente au fil, et la couche non poreuse recouvre la couche poreuse.

9. Conducteur isolé selon la revendication 6, 7 ou 8, qui a été fritté pour faire fondre les couches du matériau composite.

10. Procédé d'isolation d'un conducteur électrique comprenant l'extrusion sous forme d'une pâte un matériau d'isolation électrique formé à partir d'un mélange intime de 5 à 40% en poids d'un copolymère thermoplastique particulaire de tétrafluoroéthylène et de perfluoro(propylvinyléther) et de 60 à 95% en poids de polytétrafluoroéthylène (PFTE) de type dispersion coagulée; le calandrage du matériau et la formation d'un ruban; l'application dudit ruban autour d'un substrat conduisant l'électricité; et le frittage du matériau avant ou après l'application sur le substrat.

11. Procédé selon la revendication 10, dans lequel le matériau est fritté à une température de 350 à 450°C pendant une durée de 0,5 à 20 min.

12. Procédé d'isolation d'un conducteur électrique, qui comprend le revêtement d'un film avec deux couches adjacentes de ruban de matériau composite, une couche étant formée d'un matériau composite non poreux selon la revendication 1, et la seconde couche étant formée d'un matériau composite poreux en feuille; le matériau poreux étant formé d'une membrane poreuse de polytétrafluoroéthylène (PFTE) expansé et d'un copolymère thermoplastique de tétrafluoroéthylène et de perfluoro(propylvinyléther), dans lequel au moins une partie du copolymère thermoplastique est noyée à l'intérieur des pores du polytétrafluoroéthylène poreux, et le frittage du matériau pour faire fondre les couches en une structure unitaire.
